# EUROPEAN PATENT SPECIFICATION

(11) **EP 1 521 128 B1**
(45) Date of publication and mention of the grant of the patent: **05.08.2009**
(21) Application number: 04104732.5
(22) Date of filing: 28.09.2004
(51) Int. Cl.: G03G 9/09

(54) **Coloured magnetically attractable toner powder**
Magnetisches Farbtonerpulver
Poudre de révélateur magnétique colorée

(30) Priority: 30.09.2003 NL 1024415
(43) Date of publication of application: 06.04.2005
(73) Proprietor: Océ-Technologies B.V., 5914 CC Venlo (NL)
(72) Inventor: Coppenrath, Marcella, 5768 CL Meijel (NL); Everaars, Marcel D., 5985 PX Grashoek (NL); Ickenroth, Paul J.G., 6071 LM Swalmen (NL); Smits, Huberdina P.M., 5809 AL Leunen (NL)
(74) Representative: Janssen, Paulus J. P.

(56) References cited:
- EP-A- 0 350 099
- US-A- 5 482 805
- US-A- 5 693 445

## Description

The invention relates to coloured magnetically attractable toner powder of the type described in European Patent Specification No. 0 350 099. This type of toner powder is specifically adapted for use in an electrophotographic printing or copying machine, as described, inter alia, in US Patent 4 860 035 and European Patent 0 373 704.

The toner powder described in European Patent 0 350 099 contains magnetically attractable material enclosed by or dispersed in a colouring substance which contains thermoplastic resin and colouring material, fluorescent dye, particularly a mixture of yellow and red or magenta fluorescent dye, being present as colouring material. Although according to this patent specification it is possible to obtain toner powders with a reasonably good colour quality, a full colour printing system in particular requires improved toner powders in the colours red and magenta. There is particularly a need for red toner powder having a much higher chroma, hence higher colour saturation, than the red toner powders described in the above patent specification or that can be obtained with the combinations of yellow and red or magenta fluorescent dye described therein.

In United States Patent 5,482,805 a toner is described comprised of resin particles, magnetite, carbon black, rhodamine charge additive, wax, and a surface mixture of aluminium oxide, strontium titanate and a polyvinylidene fluoride.

The invention relates to coloured magnetically attractable toner powder, the separate particles of which consist of magnetically attractable material enclosed by a colouring substance, or finely divided therein, wherein the colouring substance contains thermoplastic resin and a mixture of fluorescent dyes and is **characterised in that** the mixture of fluorescent dyes contains a dye of the formula I:

Dyes of this formula are known per se under Colour Index No. C1 Pigment Red 81:1.

Using a dye according to the above formula I, it is possible to obtain red and magenta coloured toner powders with a considerably higher colour saturation than the toner powders that could be obtained hitherto using red or magenta coloured dyes as mentioned in European Patent Specification 0 350 099. Like the dye CI Basic Violet 11:1 (Basonyl Rot 550), the dyes according to the above formula are fluorescent.

To manufacture a red toner powder, the dye according to the above formula is combined with one or more highly yellow fluorescing dyes, as described in the above-mentioned European Patent 0 350 099. Furthermore, in order to obtain the correct colour shade, one or more other red dyes can be added in addition to red dye according to the above formula. Apart from improved red and magenta coloured toner powders, considerably improved yellow toner powders can also be obtained according to the invention, by adding to the colouring substance not only yellow fluorescent dye but also a small quantity of the dye according to the above formula I. The toner powders according to the invention can be prepared in a known manner by dissolving the fluoresent dyes in the thermoplastic resin or mixture of thermoplastic resins or dividing the same very finely therein, and also including the magnetically attractable material therein in a finely divided state. After cooling to a solid mass, the solid mass is then processed by milling and screening to form toner powder having the required particle size which, for example, is between 9 and 14 micrometers. To make the toner powder particles suitable for use in an electrographic printing process as described in US 4 860 035, they are also made electrically conductive, for example by depositing on their surface a thin colourless electrically conductive layer. This layer can, for example, consist of fluorine-doped tin oxide and be deposited on the toner powder particles in the manner described in US Patent 5 202 211.

The raw materials for the toner powder according to the invention may be the same as described in European Patent 0 350 099.

A suitable magnetically attractable powder is carbonyl iron having an average particle size of about 3 micrometers.

The thermoplastic resin or mixture of thermoplastic resins is so selected that the fluorescent dyes used, particularly yellow and red or magenta fluorescent dyes, exhibit a high fluorescence therein. Suibtale combinations of the thermoplastic resin and (yellow) fluorescent dye can be determined in the manner described in European Patent No. 0 350 099. Suitable thermoplastic resins are epoxy resins, polyester resins and modified polyester resins which in their polymer chain bear groups with a dipole moment greater than 2, such as sulphanyl, amide, anhydride or ureide groups. Suitable epoxy resins are relatively low molecular epoxy resins such as those obtainable under the trade narmes Epikote 1001 and 1004 (Shell-Nederland). Also usable are the resins derived from such epoxy resins and obtained by blocking the epoxy groups with a monofunctional reagent such as p-cumyl phenol, or blocking them to a large extent with such a monofunctional reagent and otherwise cross-linking them by intermolecular reaction and/or reaction with a polyfunctional epoxy hardener. Suitable thermoplastic resins derived from epoxy resins are described, for example, in UK Patent Specifications 2007382, 2014325 and 203653. These resins are regarded as epoxy resins in the context of the invention. Applicable polyester resins are linear resins derived from a dicarboxylic acid and a diol, and also branched polyester resins obtained by polymerisation of a dicarboxylic acid with a mixture of a diol with a small quantity, for example 5 mol-%, of a more than bivalent alcohol or by polymerisation of a diol with a mixture of a dicarboxylic acid with a small quantity of a more than bivalent carboxylic acid. Suitable polyester resins are described inter alia in Netherlands Patent Applications 6807896 and 7116891 and European Patent Application 146980.
Polyester resins or modified polyester resins which in their polymer chain bear groups with a dipole moment greater than 2 can be obtained by including in the reaction mixture in a suitable quantity, for example 10 to 50 mol-%, a bifunctional or polyfunctional reagent which bears such polar groups or forms such groups during the polymerisation reaction. Thus sulphonyl groups can be incorporated in the polymer chain by adding to the reaction mixture a diol which bears sulphonyl groups, as described in Netherlands Patent Application 7116891. Modified polyester resins which bear amide groups in their polymer chain (hereinafter referred to as polyester amides) can be obtained by the standard polycondensation techniques for the preparation of polyesters, the diol in the reaction mixture being partly replaced (for example 10 to 50 mol-%) by a diamine or amino-alcohol.

Examples of suitable diamines and amino-alcohols are tetramethylene diamine, hexamethylene diamine, p-phenylene diamine, 1-amino-2-ethanol, 1-amino-2-propanol and 1-amino-3-propanol.

The colouring material contains at least one dye according to the above formula, wherein the anion X^{⊖} can be varied in order thus to optimise the solubility or miscibility of the dye in thermoplastic resin. Generally, the solubility of the dye in the above-mentioned resins can be improved by using the dye in the form of the tetrafluoroborate, borofluoride, perchlorate, hexafluoro-zirconate or ethyl sulphate instead of the form current in the art, as a chloride, fluoride or sulphate.

For a magenta toner powder, the above dye, in order to obtain the correct colour shade, can advantageously be combined with a red-violet fluorescent dye of the type C.I. Basic Violet 11:1 (C.I. 45174). For a red toner powder, a highly yellow fluorescing dye, a mixture of such dyes or a mixture of such dye with one or more yellow pigments is added to the magenta colour formulation. Suitable yellow fluorescent dyes are Macrolex Fluorescent Yellow 10GN (C.I. Solvent Yellow 160:1), Thermoplast f-Gelb 084 (C.I. nr. 59075), Hostasol Gelb 3G (C.I. Solvent Yellow 98), Macrolex Orange R (C.I. Disperse Orange 47) and Maxilon Brilliant Flavine 10GFF (C.I. Basic Yellow 40).

The total quantity of fluorescent dye in toner powder according to the invention depends on the colour gradation and colour saturation required. Generally, the best results are already obtained with a relatively low total quantity of colouring material which, calculated on the basis of the quantity of thermoplastic resin, amounts to not more than about 1.5 to 4% by weight. In addition to thermoplastic resin, fluorescent dyes and magnetically attractable material, toner powder according to the invention can have further additives in order to influence specific properties. Thus, other (non-fluorescent) dyes or pigment can be added to obtain a desired colour shade. White pigment, for example titanium oxide or zinc oxide, can be added in order to mask the dark colour of the magnetically attractable material. A metal salt with a diamagnetic anion can be added in order to avoid fluorescence quenching of the fluorescent dyes.

The invention will now be explained with reference to the following examples.

The values for L* (lightness), C* (chroma) and h (hue) given in these examples for the toner powders are all obtained by measuring a compact toner powder mass in a cuvette. The value L* particularly of the toner powders described hereinafter and already belonging to the prior art may therefore appear lower than the L* value previously indicated in the literature for these toner powders or toner powders which are comparable in respect of composition. All the colour values indicated hereinafter were determined in the same way and are therefore satisfactorily comparable with one another. In addition, the results obtained according to the invention are also visually well perceptible. The colour measurements of the toner powders were carried out with the Coloreye 7000A colorimeter made by Gretag Macbeth with the CIE D65 illuminant as light source. The measurements were carried out on a clean quartz glass cuvette filled with 7 g of toner powder. The cuvette had a diameter of 60 mm and a height of 40 mm (supplied by Minolta).

The reflection spectrum of the toner powder material was measured and then L*, C* and h were calculated therefrom.

The measurements of the Coloreye 7000A are distinguished by good reproducibility and the possibility of carrying out measurements on a relatively thick powder layer so that the colour of the powder itself is actually determined and any ambient influences are excluded. The same clean cuvette was of course used for all the colour measurements.

### Comparative Example 1

Comparative example with the best possible formulations in respect of colour quality for magenta, red and yellow toner powder without a dye according to the invention.

All the toner powders (including those according to the invention described in Examples 2, 3 and 4) were prepared in the same way by mixing a powder mixture of thermoplastic resin, magnetisable material and colouring constituents in an extruder for about 1 hour at 110°C, processing the extruded material after cooling, by milling and screening, to give toner powder with the particle size between about 9 and 14 micrometers.

| *A Magenta toner powder* | |
|---|---|
| 83.3 % by weight | Polyester resin derived from propoxylated bisphenol A and adipic acid/isophthalic acid in a 1/3 ratio by weight |
| 15 % by weight | Carbonyl iron with a specific weight per unit area of 0.55 m²/g |
| 1.7 % by weight | Basonyl Rot 550 - tetrafluoroborate (Colour Index No. 45174) |
| Colour values: | L* : 32.9 ; C* : 46.1 ; h : 349.7 |

| *B Red toner powder* | |
|---|---|
| 80.6 % by weight | Polyester resin derived from propoxylated bisphenol A and adipic acid/isophthalic acid in a 1/3 ratio by weight |
| 15 % by weight | Carbonyl iron with a specific weight per unit area of 0.55 m²/g |
| 2.9 % by weight | Paliogeen Rood K3580 (Colour Index No. 71137) |
| 0.95 % by weight | Basonyl Rot 550 - tetrafluoroborate |
| 0.55 % by weight | Macrolex Fluorescent Yellow 10GN (Colour Index: Solvent Yellow 160:1) |
| Colour values: | L* : 30.3 ; C* : 46.8 ; h : 34.6 |

| *C Yellow toner powder* | |
|---|---|
| 94.9 % by weight | Polyester resin derived from propoxylated bisphenol A and adipic acid/isophthalic acid in a 1/3 ratio by weight |
| 3 % by weight | Carbonyl iron with a specific weight per unit area of 0.55 m²/g |
| 0.6 % by weight | Macrolex Fluorescent Yellow 10GN (Colour Index: Solvent Yellow 160:1) |
| 1.5 % by weight | Hostasol Gelb 3G (Colour Index: Sovlent Yellow 98) |
| Colour values: | L* : 62,5 ; C* : 77,6 ; h : 92,3 |

### Example 2

| *Magenta toner powder* | |
|---|---|
| 83.65 % by weight | Polyester resin derived from propoxylated bisphenol A and adipic acid/isophthalic acid in a 1/3 ratio by weight |
| 15 % by weight | Carbonyl iron with a specific weight per unit area of 0.55 m²/g |
| 0.45 % by weight | Basonyl Rot 550 tetrafluoroborate |
| 0.9 % by weight | Dye of formula I in the form of the ethyl sulphate |
| Colour values: | L* : 38.1 ; C* : 50.5 ; h : 359.4 |

### Example 3

| *Red toner powder* | |
|---|---|
| 82.35 % by weight | Polyester resin derived from propoxylated bisphenol A and adipic acid/isophthalic acid in a 1/3 ratio by weight |
| 15 % by weight | Carbonyl iron with a specific weight per unit area of 0.55 m²/g |
| 0.45 % by weight | Basonyl Rot 550 tetrafluoroborate |
| 0.87 % by weight | Formula I dye as ethyl sulphate |
| 0.84 % by weight | Macrolex Fluorescent Yellow 10GN |
| 0.49 % by weight | Hostasol Gelb 3G |
| Colour values: | L* : 37.7 ; C* : 59.9; h : 41.8 |

### Example 4

| *Yellow toner powder* | |
|---|---|
| 94.89 % by weight | Polyester resin derived from propoxylated bisphenol A and adipic acid/isophthalic acid in a 1/3 ratio by weight |
| 3 % by weight | Carbonyl iron with a specific weight per unit area of 0.55 m²/g |
| 0.6 % by weight | Macrolex Fluorescent Yellow 10GN |
| 1.49 % by weight | Hostasol Gelb 3G |
| 0.02 % by weight | Formula I dye as ethyl sulphate |
| Colour values: | L* : 68.3 ; C* : 89.5; h : 88.3 |

### Example 5

Toner powders according to the above examples were processed, in the manner described in US Patent 5 202 211, Example 5, by coating with fluorine-doped tin oxide, to give electrically conductive toner powders having a resistance of about 10⁵ ohm.m (measured as described in US Patent 5 202 211). Using these toner powders, coloured surfaces were printed in an Océ CPS 700 colour printer on receiving paper of type Océ Top Colour Paper, CC520, white, 100g/m².

The colour values of the printed colour surfaces on the prints were as follows:
Magenta in accordance with example 1:L* = 48 C* = 66 h = 330
Magenta in accordance with example 2:L* = 52 C* = 68 h = 340
Red in accordance with example 1:L* = 43 C* = 61 h = 30
Red in accordance with example 3:L* = 50 C* = 68 h = 37
Yellow in accordance with example 1:L* = 81 C* = 94 h = 93
Yellow in accordance with example 4:L* = 84 C* =100 h = 91

## Claims

1. A coloured magnetically attractable toner powder containing magnetically attractable material and a colouring substance containing thermoplastic and colouring constituents, **characterised in that** the colouring constituents comprise a mixture of fluorescent dyes, at least one of said fluorescent dyes satisfying the formula: where X is an anion.

2. A toner powder according to claim 1, **characterised in that** the anion is a tetrafluoroborate, perchlorate, hexafluorozirconate or ethyl sulphate anion.

3. A toner powder according to claim 1, **characterised in that** the mixture of fluorescent dyes comprises a yellow fluorescent dye.

4. A toner powder according to any one or more of the preceding claims, **characterised in that** the mixture of fluorescent dyes further contains red or magenta fluorescent dye.

5. A toner powder according to claim 4, **characterised in that** the dye is C.I. Basic Violet 11:1 (C.I. 45174).

## Patentansprüche

1. Gefärbtes, magnetisch anziehbares Tonerpulver, das magnetisch anziehbares Material und eine färbende Substanz mit thermoplastischen und färbenden Bestandteilen enthält, **dadurch gekennzeichnet, daß** die färbenden Bestandteile ein Gemisch aus fluoreszierenden Farbstoffen umfassen und wenigstens einer dieser fluoreszierenden Farbstoffe der folgenden Formel genügt: wobei X ein Anion ist.

2. Tonerpulver nach Anspruch 1, **dadurch gekennzeichnet, daß** das Anion ein Tetrafluorborat-, Perchlorat-, Hexafluorzirkonat- oder Ethylsulfat-Anion ist.

3. Tonerpulver nach Anspruch 1, **dadurch gekennzeichnet, daß** das Gemisch aus fluoreszierenden Farbstoffen einen gelben fluoreszierenden Farbstoff umfaßt.

4. Tonerpulver nach einem oder mehreren der vorstehenden Ansprüche, **dadurch gekennzeichnet, daß** das Gemisch aus fluoreszierenden Farbstoffen weiterhin einen fluoreszierenden Farbstoff in rot oder magenta enthält.

5. Tonerpulver nach Anspruch 4, **dadurch gekennzeichnet, daß** der Farbstoff C.I. Basic Violet 11:1 (C.I. 45174) ist.

## Revendications

1. Poudre de toner colorée magnétiquement attirable, contenant un matériau magnétiquement attirable et une substance colorante contenant des constituants thermoplastiques et colorants, **caractérisée en ce que** les constituants colorants comprennent un mélange de colorants fluorescents, au moins l'un des dits colorants fluorescents satisfaisant à la formule : dans laquelle X est un anion.

2. Poudre de toner selon la revendication 1, **caractérisée en ce que** l'anion est un anion tétrafluoroborate, perchlorate, hexafluorozirconate ou éthyl sulfate.

3. Poudre de toner selon la revendication 1, **caractérisée en ce que** le mélange de colorants fluorescents comprend un colorant fluorescent jaune.

4. Poudre de toner selon l'une ou plusieurs quelconques des revendications précédentes, **caractérisée en ce que** le mélange de colorants fluorescents contient, en outre, un colorant fluorescent rouge ou magenta.

5. Poudre de toner selon la revendication 4, **caractérisée en ce que** le colorant est le violet basique C.I. 11 : 1 (C.I. 45174).
